

Jan. 26, 1965

3,167,411

J. J. BIALY ET AL.  
ANTI-ICING JET FUEL COMPOSITION CONTAINING  
A HEXAALKYL PHOSPHORIC TRIAMIDE

Filed Feb. 28, 1962



1

3,167,411

ANTI-ICING JET FUEL COMPOSITION CONTAINING A HEXAALKYL PHOSPHORIC TRIAMIDE

Jerzy J. Bialy, Beacon, and George W. Eckert, Wappingers Falls, N.Y., assignors to Texaco Inc., New York, N.Y., a corporation of Delaware

Filed Feb. 28, 1962, Ser. No. 176,237

5 Claims. (Cl. 44-72)

This invention relates to a novel fuel composition. More particularly, the invention relates to turbine or jet fuels having outstanding anti-icing properties. This improvement is based on the effect of an anti-icing additive consisting of a polyalkyl phosphoric triamide.

Reliability of the fuel supply under extremely severe operating conditions is a matter of paramount importance in the operation of turbine or jet engine aircraft. It is also essential that the fuel supply be absolutely free of any suspended solid particles in order not to block or impair the operation of the fuel atomizer and other fine components in the jet engine. The provision of uncontaminated fuel free of solid particles to the engine is assured by passing the fuel through exceedingly fine filters in order to screen out any contained solid particles.

Jet fuels always contain minor amounts of water dissolved in the fuel itself. When proper care has not been taken in the handling of the fuel, water in excess of the amount dissolved in the fuel will often be present. Jet engine aircraft frequently encounter extremely low-temperature operating conditions which cause the water in the fuel to form ice, generally in the form of small crystals. These ice crystals are caught by the fuel filter initially restricting and finally preventing passage of the fuel therethrough resulting in engine failure from the lack of fuel.

A fuel composition has now been discovered which inhibits or prevents the formation of ice from the water contained therein even under extremely low temperatures. This is achieved by the addition of very small amounts of an additive composition which imparts exceptionally good anti-icing properties to jet fuel compositions.

In accordance with this invention, there is provided a jet fuel composition containing 0.02 to 0.35 weight percent of a polyalkyl phosphoric triamide. Polyalkyl phosphoric triamides are represented by the formula:



in which R and R' each represent alkyl radicals having from 1 to 4 carbon atoms.

The preferred polyalkyl phosphoric triamide anti-icing additives of the invention are the hexaalkyl phosphoric triamides, such as hexamethyl phosphoric triamide, hexethyl phosphoric triamide, hexabutyl phosphoric triamide, hexapropyl phosphoric triamide and the like. Mixed hexaalkyl phosphoric triamides are also effective as the anti-icing additive. The preferred additive of this invention is hexamethyl phosphoric triamide.

The anti-icing additive of this invention is employed in turbine or jet engine fuel compositions. The fuels are made up of straight run or cracked hydrocarbon components in the gasoline and kerosene boiling ranges, i.e., boiling from about 100 to about 600° F. Commercial JP-4 type jet fuel, which consists of about 65 percent gasoline and 35 percent middle distillate, is typical of the fuels improved by the anti-icing additive of the invention.

2

The jet fuel of the invention is conveniently prepared by mixing the base fuel with the polyalkyl phosphoric triamide. As noted above, the jet fuel will generally contain from about 0.02 to 0.35 weight percent of the additive. The preferred range of proportions for the additive, however, are from about 0.05 to 0.20 weight percent.

An important feature of this invention is that the outstanding anti-icing properties imparted to the fuel are obtained with relatively small amounts of the additive. Whereas heretofore, jet fuel anti-icing additives have been proposed in amounts of 0.5 to 1 percent or more, the present additive gives the desired properties with a very small amount of additive. For most purposes, effective anti-icing is obtained at about 0.10 weight percent of the additive.

The single figure is a schematic diagram of a test system for determining the pumpability temperature of fuels at low temperatures.

The temperature at which the flow rate of the fuel can no longer be maintained and/or substantial pressure drop develops across the screen is defined as the pumpability temperature.

Water-containing jet fuels of the invention were tested for their pumpability properties at low temperature. Basically, the test involved circulating the fuel in a closed system containing a fine metal screen filter while gradually reducing the temperature of the fuel. Sensitive temperature and pressure devices placed on the inlet and outlet sides of the filter indicated the temperature at which a substantial pressure drop was brought about by the formation of ice in the fuel.

Two criteria of additive performance were employed in the test:

(1) Concentration of additive to yield -76° F. pumpability temperature with water-saturated fuel, and

(2) Concentration of additive to yield -45° F. pumpability temperature with water-saturated fuel to which 2 cc. per gallon of free water was added.

Referring now to FIGURE 1 showing a diagram of the low temperature pumpability test system, 10 is a reservoir for the fuel sample. In the test system employed, this reservoir had a capacity of four liters. Conduit 11 connects the fuel reservoir with a pump 12, and flow meter 13 which controls the rate of flow of the fuel. The test fuel is passed through conduit 14 into cooling coil 15 which is immersed in a low temperature cooling bath in vessel 16. The temperature of the cooling bath is registered by temperature means 17 and is controlled by circulation from cooling liquid reservoir 18 and inlet and return circulating conduits 19 and 20 respectively. The test fuel is passed through conduit 21 into filtering device 22 which has a 200 mesh screen filter 23 mounted therein for filtering the fuel. Conduit 24 is a return line for the fuel to the sample reservoir. The filter device is equipped with temperature indicating means 25 and 26 to indicate the temperature on the inlet and outlet sides of the filtering device respectively. This device is also equipped with a sensitive pressure means 27 to show the pressure differential between that in the inlet conduit leading into the filter and the pressure in the outlet conduit from the filter. The pressure device is sensitive to a pressure differential of  $\pm 1$  mm. of mercury. Plugging of the filter caused by ice formation is indicated by a sharp pressure drop across the filter.

Cooling liquid reservoir 18 contains a Dry Ice-acetone mixture which is circulated around the test cooling coil in vessel 16. Steady cooling of the test fuel is obtained by controlling the flow of cooling liquid through conduits 19 and 20.

The jet fuel employed for testing the additive of the invention had the inspection tests listed in Table I below:

**TABLE I**  
*Fuel Inspection Tests*

|                                  |          |
|----------------------------------|----------|
| Gravity, ° API                   | 52.8     |
| Freezing point, ° F.             | Below 76 |
| Luminometer number               | 62.8     |
| Hydrocarbon group analysis, FIA: |          |
| Saturates                        | 89       |
| Aromatics                        | 10       |
| Olefins                          | 1        |
| RVP                              | 2.3      |
| ASTM distillation:               |          |
| IBP                              | 135      |
| 5%                               | 173      |
| 10%                              | 188      |
| 20%                              | 212      |
| 30%                              | 237      |
| 40%                              | 263      |
| 50%                              | 292      |
| 60%                              | 321      |
| 70%                              | 348      |
| 80%                              | 398      |
| 90%                              | 457      |
| 95%                              | 485      |
| EP                               | 509      |
| Recovered                        | 98.8     |
| Loss                             | 1.1      |
| Residue                          | 0.4      |

The test procedure followed involves adding 4 liters of the test fuel to the reservoir which is thereafter stoppered to prevent the entrance of water from condensation during the cooling period. The circulating pump is started and air is purged from the manometer lines and filter screen housing via vents provided for this purpose. The fuel flow rate is adjusted to 0.67 g.p.m. (gallons per minute). At the start of the cooling cycle, the Dry Ice compartment is filled with Dry Ice and the cold acetone-Dry Ice solution is circulated to the main bath which contains the cooling coils of the fuel test circuit. Dry Ice is dropped into the cooling bath initially in quantities sufficient to cool the fuel rapidly to 20° F., then in an amount to cool the fuel at the rate of about 0.5° F. per minute. The temperature of the cooling bath is further controlled by controlling the flow of the cooling liquid.

When the first appreciable rise (5 to 10 mm. Hg) in screen pressure differential occurs, the temperature prevailing at that time is maintained for at least 5 minutes while maintaining the fuel flow at 0.67 g.p.m. If the differ-

5. tial pressure continues to increase at this temperature to the point where flow can no longer be maintained, this is taken as the pumpability temperature. If the pressure differential does not continue to rise, the temperature is decreased in 1° F. increments until a large increase in pressure differential occurs.

The pumpability temperature for a water-saturated JP-4 fuel is usually between 5 and 15° F. With 2 ml. per gallon of free water, the pumpability temperature is generally in the range of 10 to 20° F.

A jet fuel having the Inspection Tests shown in Table I was tested for its pumpability temperatures in the test device and manner described hereinabove. The anti-icing additive employed consisted of hexamethyl phosphoric triamide. The tests were conducted on a fuel saturated with water and also on a fuel saturated with and containing excess water in the amount of 2 ml. of excess water per gallon of fuel.

At a hexamethyl phosphoric triamide concentration of 0.1 weight percent, the fuel saturated with water had a pumpability temperature of  $-76^{\circ}\text{ F}$ .

At a hexamethyl phosphoric triamide concentration of 0.1 weight percent, the fuel saturated with water and containing 2 ml. of excess water per gallon of fuel also had a pumpability temperature of  $-76^{\circ}$  F.

We claim:

gasoline and kerosene hydrocarbon fractions boiling from about 100-600 degrees F., said hydrocarbon fractions being free of alkyl lead anti-knock compounds, and (2) an anti-icing amount of a hexaalkyl phosphoric triamide in which said alkyl radicals have from 1 to 4 carbon atoms.

2. A jet fuel composition according to claim 1 containing 0.02 to 0.35 weight percent of said hexaalkyl phosphoric triamide.

3. A jet fuel composition according to claim 1 in which said triamide is hexamethyl phosphoric triamide.

4. A jet fuel composition according to claim 1 containing from about 0.05 to 0.20 weight percent of said hexa-  
40 alkyl phosphoric triamide.

5. A jet fuel composition according to claim 4 in which said hexaalkyl phosphoric triamide is hexamethyl phosphoric triamide.

**References Cited in the file of this patent**

UNITED STATES PATENTS

|           |                         |                |
|-----------|-------------------------|----------------|
| 2,765,220 | Yust et al. -----       | Oct. 2, 1956   |
| 2,863,743 | Pellegrini et al. ----- | Dec. 9, 1958   |
| 2,897,068 | Pellegrini -----        | July 28, 1959  |
| 2,974,022 | Lindstrom et al. -----  | Mar. 7, 1961   |
| 2,999,739 | Heron -----             | Sept. 12, 1961 |